# EUROPEAN PATENT SPECIFICATION

(11) **EP 1 574 587 B1**
(45) Date of publication and mention of the grant of the patent: **16.07.2008**
(21) Application number: 03780855.7
(22) Date of filing: 17.12.2003
(51) Int. Cl.: C21D 8/00, C22C 38/00, C22F 1/00, C22C 38/34, C22C 38/48

(54) **METHOD OF THERMO-MECHANICAL-TREATMENT FOR Fe-Mn-Si SHAPE-MEMORY ALLOY DOPED WITH NbC**
VERFAHREN ZUR THERMOMECHANISCHEN BEHANDLUNG FÜR EINE MIT NbC DOTIERTE Fe-Mn-Si-FORMGEDÄCHTNISLEGIERUNG
PROCEDE DE TRAITEMENT THERMO-MECANIQUE POUR ALLIAGE FE-MN-SI A MEMOIRE DE FORME DOPE AU NBC

(30) Priority: 18.12.2002 JP 2002367062
(43) Date of publication of application: 14.09.2005
(73) Proprietor: National Institute for Materials Science, Tsukuba-shi, Ibaraki 305-0047 (JP)
(72) Inventor: KIKUCHI, T., c/o NAT. INSTITUTE FOR MAT. SCIENCE, Tsukuba-shi, Ibaraki 305-0047 (JP); KAJIWARA, Satoshi, Ibaraki 305-0031 (JP); BARUJ, A., c/o NAT. INSTITUTE FOR MAT. SCIENCE, Tsukuba-shi, Ibaraki 305-0047 (JP); OGAWA, K., c/o NAT. INSTITUTE FOR MAT. SCIENCE, Tsukuba-shi, Ibaraki 305-0047 (JP); SHINYA, N., c/o NAT. INSTITUTE FOR MAT. SCIENCE, Tsukuba-shi, Ibaraki 305-0047 (JP)
(74) Representative: Vossius & Partner
(86) International application number: PCT/JP2003/016189
(87) International publication number: WO 2004/055222

(56) References cited:
- EP-A- 1 123 983
- EP-A- 1 348 772
- JP-A- 62 112 720
- US-A- 5 032 195
- US-A- 5 173 131
- US-A1- 2001 023 723
- BARUJ A ET AL: "EFFECT OF PRE-DEFORMATION OF AUSTENITE ON SHAPE MEMORY PROPERTIES IN FE-MN-SI-BASED ALLOYS CONTAINING NB AND C" MATERIALS TRANSACTIONS. JIM, SENDAI, JP, vol. 43, no. 3, March 2002 (2002-03), pages 585-588, XP009012787 ISSN: 0916-1821
- DATABASE INSPEC [Online] THE INSTITUTION OF ELECTRICAL ENGINEERS, STEVENAGE, GB; 15 December 1999 (1999-12-15), KAJIWARA S: "Characteristic features of shape memory effect and related transformation behavior in Fe-based alloys" XP002357339 Database accession no. 6526328 -& ICOMAT 98. INTERNATIONAL CONFERENCE ON MARTENSITIC TRANSFORMATIONS 7-11 DEC. 1998 SAN CARLOS DE BARILOCHE, ARGENTINA, vol. A273-275, 1999, pages 67-88, XP009058192 Materials Science & Engineering A (Structural Materials: Properties, Microstructure and Processing) Elsevier Switzerland ISSN: 0921-5093
- BARUJ A ET AL: "FURTHER IMPROVEMENT IN THE SHAPE-MEMORY PROPERTIES OF FEMNSI-BASED SHAPE-MEMORY ALLOYS CONTAINING NBC PRECIPITATES" MATERIALS SCIENCE FORUM, AEDERMANNSFDORF, CH, vol. 394/395, 2 September 2001 (2001-09-02), pages 403-406, XP009012763 ISSN: 0255-5476
- SAWAGUCHI ET AL.: 'Shitsuon de incho henkeigo jiko netsushori shita Fe-28Mn-6Si-5Cr-0.5NbC gokin no keijo kioku tokusei' THE JAPAN INSTITUTE OF METALS KOEN GAIYO vol. 133, 11 October 2003, page 75, XP002981521
- BARUJ A. ET AL.: 'Shape memory behaviour and recovery strength in training-less FE-MN-SI-based SMA containing NBC' THE JAPAN INSTITUTE OF METALS KOEN GAIYO vol. 128, page 347, XP002981522

## Description

The present invention relates to a thermomechanical treatment method for a Fe-Mn-Si-based shape memory alloy with Nb, C addition. More particularly, the present invention relates to a thermomechanical treatment method for a Fe-Mn-Si-based shape memory alloy with Nb, C addition which exhibits a satisfactory shape memory effect without undergoing so-called training, providing improved performance.

It has been a long time since the Fe-Mn-Si-based shape memory alloys had been proposed and invented. However, unfortunately, the alloys of Fe-Mn-Si system may be currently in a situation that the alloys are not sufficiently used yet and not yet put to practical use. The main cause is that the alloys can not exhibit satisfactory shape memory effect without undergoing a special thermomechanical treatment called training.

Here, the training means a process sequence of repeating the following treatment several times to improve shape memory effect. The treatment consists of deforming an alloy by 2-3% at room temperature and then heating it to around 600°C higher than the reverse transformation temperature of the alloy.

In the face of the situation of prior art in which the aforementioned troublesome training is indispensable, inventors of this invention have earnestly studied aiming at developing a treatment with simple process, especially not requiring the training. As a result, the inventors have found a fact that if a small amount of Nb and C elements is applied to a particular shape memory alloy i.e. a Fe-Mn-Si-based shape memory alloy and a suitable aging heating treatment is subjected to the alloy to generate fine NbC carbides in structure of the alloy, a sufficiently satisfactory shape memory effect is obtained without undergoing the troublesome treatment called training, and thus previously filed a patent application (see Patent Document 1 = JP-Patent 3 542 754). The inventors have studied also about the thermomechanical treatments for the alloy with Nb, C addition, and they found a fact that pre-deformation in a temperature range of from 500°C to 800°C and a subsequent aging treatment lead to a further improved shape memory effect and thus also filed patent applications about this (see Patent Document 2 = JP-A-2001-296901; Patent Document 3 = JP-A-2002-79295).

We believe that the inventions proposed in the aforementioned prior applications facilitate astonishing progress in the shape memory alloy technology, contribute to put the shape memory alloy to practical use for the future, and greatly contribute to the development of industry. However, there are still some points to be improved in proposed inventions. As for the two latter prior applications (Patent Document 2, Patent Document 3), the inventions proposed in these applications are significantly meaningful because the necessary thermomechanical treatments are quite easy compared with the training and yet well improved shape memory performance of the alloy is obtained. Thus, the degree of practical use is dramatically increased. That is, the works and effects of the inventions of these applications are quite noticeable. However, there still remains a problem that the treatment process requires a heating treatment in a high temperature range of from 500°C to 800°C, which causes difficulties in most cases. It is undeniable that this point makes it difficult to put the shape memory alloys to practical use.

EP-A-1 123 983 discloses a shape memory alloy of Fe-Mn-Si system containing at least Fe, Mn and Si, wherein the alloy contains niobium carbides in the structure and the alloy is subjected to a heat treatment for homogenization at a temperature ranging from 1000°C to 1300°C and subsequently an ageing at a temperature ranging from 400°C to 1000°C to precipitate niobium carbides.

"Materials Transactions, Vol. 43, No. 3 (2002), pp. 585-588" discloses a shape memory alloy of Fe-Mn-Si system containing Nb and C which is rolled at 870K by 6% and 14% after the solution treatment and then subjected to an ageing treatment.

"Materials Science and Engineering, A273-275 (1999), pp. 67-68" discloses a shape memory alloy of Fe-14Mn-6Si-9Cr-5Ni which is subjected to the thermomechanical treatment consisting of 10% rolling at room temperature and subsequent heating to 970 K for 10 min.

US-A-5,032,195 discloses a Fe-based shape memory alloy which is hot-rolled in the thickness of 0.8 mm and 4 mm after homogenization, and the hot-rolled plate of 4 mm is annealed at room temperature several times and then cold-rolled into a plate having 0.8 mm in thickness and the cold-rolled plate is annealed at 600°C for 2 hours.

The object of the present invention is to fundamentally solve the aforementioned problems.

The inventors of this invention has earnestly studied aiming at developing and ensuring good shape memory properties for a shape memory alloy of specified components even with deformation at low temperatures. As a result, they found that the satisfactory shape memory properties can be sufficiently ensured even with deformation at room temperature so as to achieve the aforementioned object.

That is, they found amazing fact that the excellentshape memory property of alloy can be developed just by applying a basic operation comprising deforming a Fe-Mn-Si-based shape memory alloy with Nb, C addition at room temperature and then subjecting the deformed alloy to aging heating treatment to precipitate NbC carbides. In brief, the aforementioned object is achieved by the present invention.

The present invention was made on the basis of the aforementioned knowledge and success. The object of the present invention can be achieved by the features specified in the claims.

As a thermomechanical treatment for a Fe-Mn-Si-based shape memory alloy having specified components with Nb, C addition, the deformation prior to aging is carried out in a temperature range of from 500°C to 800°C in case of the prior applications. According to the present invention, however, the deformation prior to the aging treatment can be successfully carried out not at high temperature but at room temperature, by setting the deformation ratio in a specified range.

The technical meaning of the present invention must be clearly understood as compared to the prior art and the inventions of the prior applications on which the present invention is based because there are obvious difference therebetween. That is, according to the present invention, the remarkable improvement in shape memory property is achieved first time by a combination of specified alloy components, specified deformation ratio at room temperature, and setting of aging condition to a certain range. Amazingly by run-of-the-mill thermomechanical treatment comprising a deformation at room temperature and then aging, the shape recovery ratio equivalent to that of the sample subjected to the training can be obtained and, in addition, the shape recovery stress significantly larger than that of the sample subjected to the training can be obtained. With development of the present invention, it is expected that the use of shape memory alloys will be accelerated toward the practical use in a wide variety of fields. The invention is described in detail in conjunction with the drawings, in which
Fig. 1 is a diagram showing relations between the amount of initial deformation and the shape recovery ratio depending on the thermomechanical treatment of Fe-Mn-Si-based shape memory alloys with Nb, C addition of the present invention; and
Fig. 2 is a diagram showing the relation between the recovered shape strain and shape recovery stress depending on the thermomechanical treatment of Fe-Mn-Si-based shape memory alloys with Nb, C addition of the present invention.

The reason why the deformation ratio at room temperature is specified to be from 5% to 40% comes from the fact that the deformation ratio lower than 5% does not effectively contribute to improvement in shape memory property while the deformation ratio over 40% makes a sample too hard so that it is extremely difficult to deform the sample after subjected to an aging treatment.

An alloy as to be subjected to the thermomechanical treatment method for a Fe-Mn-Si-based shape memory alloy with Nb, C addition of the present invention has the following chemical compositions, just as specified in the prior applications, 1) Mn: 15% to 40% by weight, Si: 3% to 15% by weight, Nb: 0.1% to 1.5% by weight, C: 0.01% to 0.2% by weight, and Fe and inevitable impurities: residual amount, wherein the atomic ratio Nb/C between Nb and C is 1 or more;
2) The Fe-Mn-Si-based shape memory alloy with Nb, C addition has the following compositions Mn: 15% to 40% by weight, Si: 3% to 15% by weight, Cr: 1% to 20% by weight, Nb: 0.1% to 1.5% by weight, C: 0.01% to 0.2% by weight, and Fe and inevitable impurities: residual amount, wherein the atomic ratio Nb/C between Nb and C is 1 or more; 3) The Fe-Mn-Si-based shape memory alloy with Nb, C addition has the following compositions Mn: 15% to 40% by weight, Si: 3% to 15% by weight, Cr: 1% to 20% by weight, Ni: 0.1% to 20% by weight, Nb: 0.1% to 1.5% by weight, C: 0.01% to 0.2% by weight, and Fe and inevitable impurities: residual amount, wherein the atomic ratio Nb/C between Nb and C is 1 or more.

In either of the Fe-Mn-Si-based shape memory alloys with Nb, C addition, the atomic ratio Nb/C between Nb and C in the alloy is preferably from 1.0 to 1.2.

Further, the alloy as to be subjected to a thermomechanical treatment method for the Fe-Mn-Si-based shape memory alloy of the present invention is permitted to contain, as impurities, one or more of a group consisting of Cu of 3% by weight or less, Mo of 2% by weight or less, Al of 10% by weight or less, Co of 30% by weight or less, and N of 5000 ppm or less.

Hereinafter, the invention will be specifically described on the basis of Fig. 1 and Fig. 2. It should be noted that examples shown in the drawings are for the purpose of disclosure for helping the easy understanding of the present invention and are not intended to limit the scope of the present invention.

### EXAMPLES

First, a Fe-28Mn-6Si-5Cr-0.53Nb-0.06C alloy (% by weight) with Nb, C addition of the present invention was prepared by melting. How the shape memory property is improved by rolling at room temperature and then subjecting it to an aging treatment in a temperature range of 400°C to 1000°C for a time period from 1 minute to 2 hours, is shown below.

FIG. 1 is a graph showing differences in shape recovery ratio among a case in which only aging was conducted (0% rolling) and cases in which aging was conducted after rolling by 10%, 20% and 30% at room temperature. In all of the cases, the aging treatment was conducted at 800°C for 10 minutes. For comparison, results of samples of the Fe-28Mn-6Si-5Cr alloy with no Nb, C addition prepared only by annealing and samples of the alloy prepared after subjected to the training five times are shown. The abscissa shows the initial strain (%) by tensile deformation at room temperature, and the ordinate shows the recovery ratio of strain when the sample is heated to 600°C. When heated to 400°C, approximately the same shape recovery ratio is also obtained. The samples used in tests were test pieces having a thickness of 0.6 mm, a width of 1 to 4 mm, and a length (gage length) of 15 mm.

As is known from this figure, the sample rolled by 10% has shape memory recovery ratios nearly equivalent to or slightly lower than those of the alloy with no Nb, C addition which was subjected to training five times. Practically the necessary initial strain is believed to be about 4%. A shape memory recovery ratio of about 90% shown at this strain strongly suggests that it is used as a practically applicable alloy. Training of at least five times is necessary for obtaining the same shape recovery ratio as this sample, with a conventional Fe-Mn-Si-based shape memory alloy with no Nb, C addition. As is understood from this, the present invention exhibits shape memory properties with a simple method.

The sample with a higher rolling ratio of 20% has shape memory recovery ratios nearly equivalent to or slightly higher than those of the case without rolling (only aged). However, the sample with a further higher rolling ratio of 30% has shape memory recovery ratios lower than those of the case which was only aged in a range with large initial strain.

On the other hand, as for shape recovery stress which is one of the important shape memory properties for practical use, the shape recovery stresses of samples aged after rolling by 20% and 30% are remarkably improved. Fig. 2 is a graph showing the degrees of improvement in shape recovery stress of these samples, in comparison with the case in which only aging was conducted (0% rolling) and a case in which the aging was conducted after rolling by 10%. The recovery stress when recovered strain on the abscissa is zero means the stress generated when a sample is tensile-deformed at room temperature, then, heated to the reverse transformation temperature or more in a state that the both ends of the sample are fixed without any recovery, and returned to room temperature again. The recovery stress at recovered strain of 2%, for example, means the stress generated in case that the both ends of the sample are fixed after a recovery of strain by 2%. Tests were conducted with the initial strain given at room temperature of from 4% to 6%.

The test pieces used were the same as those used for obtaining the results shown in Fig. 1. The recovered strain on the abscissa in Fig. 2 is explained, taking a case where a shape memory alloy is used as a coupling for examples. It is equivalent to the ratio (%) of clearance between the pipes and the coupling part (shape memory alloy) to the diameter. Remarkable increase in shape recovery stress is observed in a range of high rolling ratio: a shape recovery stress of 310MPa is obtained at the recovered strain of 0% when the rolling ratio is from 20% to 30% at room temperature and a shape recovery stress of 200 MPa is obtained even at the recovered strain of 2% for the same rolling ratio. It is also found that the same shape recovery stress as the case subjected to training is obtained even in a case that the rolling ratio is 10%.

That is, as is known from the results of this figure (Fig. 2), remarkable increase in shape recovery stress is observed in cases of high rolling ratios (20%, 30%) as compared to the cases of a rolling ratio of 0% and a rolling ratio of 10%. For the sake of comparison, Fig. 2 shows shape recovery stresss of the sample with no Nb, C addition and the sample subjected to the training five times. It is seem from this figure that the recovery stresses of these samples are much smaller than those of the present invention.

As described above, the present invention was made by finding that the deformation treatment prior to the aging treatment to a Fe-Mn-Si-based shape memory alloy having specified components with Nb, C addition can be successfully carried out at room temperature if the deformation ratio is in a specified range. The technical meaning of the present invention must be clearly understood because there are obvious advantages as compared to a conventional one which requires the training accompanied by troublesome operation and the inventions of the prior applications which still require high-temperature deformation in a range of from 500°C to 800°C.

That is, according to the present invention, the remarkable improvement in shape memory property is achieved first time by a combination of specified alloy components, specified deformation ratio at room temperature, and setting of aging condition to a certain range. Amazingly by run-of-the-mill thermomechanical treatment comprising a deformation at room temperature and then aging, the shape recovery ratio equivalent to that of the sample subjected to the training can be obtained and, in addition, the shape recovery stress significantly larger than that of the sample subjected to the training can be obtained. Anyway, the meaning of the present invention is significant. The shape memory alloy according to the present invention can be used as tightening materials for various applications, for example, for tightening water pipes, tightening oil pipes, etc., which will produce great economic effects.

It should be noted that the applications as tightening materials mentioned above are just examples and the present invention is not limited to such applications. With the development of the present invention, it is expected that the shape memory alloy will be put to practical use for various applications in a wide variety of fields.

The present invention provides a thermomechanical treatment means for a Fe-Mn-Si-based shape memory alloy having specified components with Nb, C addition with simple processing treatment prior to aging. In case of the prior applications, the deformation treatment prior to aging is carried out in a temperature range of from 500°C to 800°C. According to the present invention, however, the deformation treatment prior to the aging treatment can be successfully carried out not at high temperature but at room temperature, if the deformation ratio in a specified range.

The technical meaning of the present invention must be clearly understood as compared to the prior art and the inventions of the prior applications because there are obvious difference therebetween. That is, according to the present invention, the remarkable improvement in shape memory property is achieved first time by a combination of specified alloy components, specified processing ratio at room temperature, and setting of aging condition into a certain range.

The technical meaning of the present invention must be clearly understood as compared to the prior art and the inventions of the prior applications because there are obvious difference therebetween. That is, according to the present invention, the remarkable improvement in shape memory property is achieved first time by a combination of specified alloy components, specified deformation ratio at room temperature, and setting of aging condition to a certain range. Amazingly by run-of-the-mill thermomechanical treatment comprising a deformation at room temperature and then aging, the shape recovery ratio equivalent to that of the sample subjected to the training can be obtained and, in addition, the shape recovery stress significantly larger than that of the sample subjected to the training can be obtained. With development of the present invention, it is expected that the use of shape memory alloys will be accelerated toward the practical use in a wide variety of fields.

## Claims

1. A thermomechanical treatment method for a Fe-Mn-Si-based shape memory alloy with Nb, C addition, the Fe-Mn-Si-based shape memory alloy with Nb, C addition comprising, as alloy components, Mn: 15% to 40% by weight, Si: 3% to 15% by weight, Nb: 0.1% to 1.5% by weight, C: 0.01% to 0.2% by weight, optionally one or two of Cr: 1% to 20% by weight and Ni: 0.1% to 20% by weight and the balance of Fe and inevitable impurities, wherein the atomic ratio Nb/C between Nb and C is 1 or more, **characterized in that** the method comprises the steps of
deforming a Fe-Mn-Si-based shape memory alloy with Nb, C addition by a deformation ratio of from 5% to 40% at room temperature, and
subjecting the deformed alloy to aging heating treatment to precipitate NbC carbides.

2. A thermomechanical treatment method for a Fe-Mn-Si-based shape memory alloy with Nb, C addition as claimed in claim 1, wherein the atomic ratio between Nb and C is set in a range of from 1.0 to 1.2.

3. A thermomechanical treatment method for a Fe-Mn-Si-based shape memory alloy with Nb, C addition as claimed in claim 1 or 2, wherein the Fe-Mn-Si-based shape memory alloy with Nb, C addition contains, as impurities, Cu: 3% by weight or less, Mo: 2% by weight or less, Al: 10% by weight or less, Co: 30% by weight or less, and/or N: 5000 ppm or less.

4. A thermomechanical treatment method for a Fe-Mn-Si-based shape memory alloy with Nb, C addition as claimed in any one of claims 1 through 3, wherein the conditions for the aging heating treatment are a temperature range of 400°C to 1000°C and a time period from 1 minute to 2 hours.

## Patentansprüche

1. Thermomechanisches Behandlungsverfahren für eine Fe-Mn-Si-basierte Formgedächtnislegierung mit Nb- und C-Zugabe, wobei die Fe-Mn-Si-basierte Formgedächtnislegierung mit Nb- und C-Zugabe als Legierungskomponenten aufweist: Mn: 15 bis 40 Gew.-%, Si: 3 bis 15 Gew.-%, Nb: 0,1 bis 1,5 Gew.-%, C: 0,01 bis 0,2 Gew.-%, optional Cr: 1 bis 20 Gew.-% und/oder Ni: 0,1 bis 20 Gew.-% und als Rest Eisen und unvermeidliche Verunreinigungen, wobei das Atomverhältnis Nb/C zwischen Nb und C mindestens 1 beträgt,
**dadurch gekennzeichnet, daß** das Verfahren die Schritte aufweist:
Verformen der Fe-Mn-Si-basierten Formgedächtnislegierung mit Nb- und C-Zugabe durch ein Formänderungsverhältnis von 5 % bis 40 % bei Raumtemperatur, und
Unterziehen der verformten Legierung einer Wärmealterungsbehandlung, um NbC-Carbide auszuscheiden.

2. Thermomechanisches Behandlungsverfahren für eine Fe-Mn-Si-basierte Formgedächtnislegierung mit Nb- und C-Zugabe nach Anspruch 1, wobei das Atomverhältnis zwischen Nb und C in einem Bereich von 1,0 bis 1,2 festgelegt ist.

3. Thermomechanisches Behandlungsverfahren für eine Fe-Mn-Si-basierte Formgedächtnislegierung mit Nb- und C-Zugabe nach Anspruch 1 oder 2, wobei die Fe-Mn-Si-basierte Formgedächtnislegierung mit Nb- und C-Zugabe als Verunreinigungen enthält: Cu: höchstens 3 Gew.-%, Mo: höchstens 2 Gew.-%, Al: höchstens 10 Gew.-%, Co: höchstens 30 Gew.-% und/oder N: höchstens 5000 ppm.

4. Thermomechanisches Behandlungsverfahren für eine Fe-Mn-Si-basierte Formgedächtnislegierung mit Nb- und C-Zugabe nach einem der Ansprüche 1 bis 3, wobei die Bedingungen für die Wärmealterungsbehandlung ein Temperaturbereich von 400 °C bis 1000 °C und eine Zeitdauer von 1 Minute bis 2 Stunden sind.

## Revendications

1. Procédé de traitement thermomécanique pour un alliage à mémoire de forme à base Fe-Mn-Si avec addition de Nb, C, l'alliage à mémoire de forme à base Fe-Mn-Si avec addition de Nb, C comprenant, à titre de composants d'alliage, Mn à raison de 15 % à 40 % en poids, Si à raison de 3 % à 15 % en poids, Nb à raison de 0,1 % à 1,5 % en poids, C à raison de 0,01 % à 0,2 % en poids, en option un ou deux des éléments que sont Cr à raison de 1 % à 20 % en poids et Ni à raison de 0,1 % à 20 % en poids, le reste étant du fer et des impuretés inévitables, le rapport atomique Nb/C entre Nb et C étant égal à 1 ou plus,
**caractérisé en ce que** le procédé comprend les étapes consistant à :
déformer un alliage à mémoire de forme à base Fe-Mn-Si avec addition de Nb, C sous un rapport de déformation de 5 % à 40 % à température ambiante, et
soumettre l'alliage déformé à un traitement thermique de vieillissement pour faire précipiter les carbures NbC.

2. Procédé de traitement thermomécanique pour un alliage à mémoire de forme à base Fe-Mn-Si avec addition de Nb, C, selon la revendication 1, dans lequel le rapport atomique entre Nb et C est choisi dans une plage de 1,0 à 1,2.

3. Procédé de traitement thermomécanique pour un alliage à mémoire de forme à base Fe-Mn-Si avec addition de Nb, C, selon la revendication 1 ou 2, dans lequel l'alliage à mémoire de forme à base Fe-Mn-Si avec addition de Nb, C contient, comme impuretés : Cu à raison de 3 % en poids ou moins, Mo à raison de 2 % en poids ou moins, Al à raison de 10 % en poids ou moins, Co à raison de 30 % en poids ou moins, et/ou N à raison de 5000 ppm ou moins.

4. Procédé de traitement thermomécanique pour un alliage à mémoire de forme à base Fe-Mn-Si avec addition de Nb, C, selon l'une quelconque des revendications 1 à 3, dans lequel les conditions pour le traitement thermique de vieillissement sont une plage de température de 400° C à 1000° C et une période temporelle de 1 minute à 2 heures.
